

July 31, 1945.

R. G. JACKSON

2,380,762

MANUFACTURE OF SHEET MATERIAL

Filed March 24, 1941



Inventor.  
Ralph G. Jackson.  
Stone, Boyden & Fawcett  
Attorneys.

## UNITED STATES PATENT OFFICE

2,380,762

## MANUFACTURE OF SHEET MATERIALS

Ralph G. Jackson, Woodbury, N. J.

Application March 24, 1941, Serial No. 385,030

9 Claims. (Cl. 117—8)

This invention relates to a method of and apparatus for treating sheet material particularly of the type employed for decorative or other purposes, on floors, walls and other surfaces. By means of this method and apparatus, sheet material is provided which is of the general type described and claimed in my patents, Nos. 1,729,833 and 1,798,779; also, there is provided sheet material characterized by the uniform distribution of the penetrant in the body of the sheet.

In applying a penetrant to a sheet material for impregnation purposes, it is frequently difficult, particularly with a dense or fairly solid sheet, to obtain uniform distribution of the penetrant in pores well down in the body of the sheet. The term "pores" is used as the equivalent of "interstices" to indicate space in the sheet not occupied by non-absorbent material. For ordinary saturation purposes, for instance, a less compact sheet material is generally treated to make certain that the sheet is filled. But in such cases there is a certain loss in wearing qualities which would not be the case if the denser, more solid, type of sheet were used. Also, in applying penetrating colorings, particularly pigmented paints, a dense, solid type of sheet is apt to permit penetration of oil or solvent vehicle but not the pigment, behaving somewhat as a filter whereby surface coloring of the sheet is effected, but little or no coloring into the body of the sheet.

In the present invention, a sheet is provided with a multitude of very fine openings constituting ducts extending from a surface into the body of the sheet so that a penetrant, such as a saturant or decorative coloring material, applied to a surface of the sheet so treated, passes more freely into or through the sheet. Such pin hole piercing of the surface is preferably done by rouletting and is in contrast to perforations or any similar treatment such as requires the removal of any substantial amount of the material of the sheet in the making of the openings. Although the surface of the sheet may be hard and compact and resistant to impregnation, after the penetrant passes beneath the surfaces, it spreads laterally from a duct and into interstices that would not be reached if dependence were placed on penetration through the normal surface. Penetration takes place more readily from the sides of a duct or pin hole opening than from the normal surface of a sheet. The ducts are distributed uniformly and are spaced a predetermined distance apart depending upon the density

of the sheet and the degree of lateral spread of a penetrant. The more dense the sheet the shorter the distance between the ducts.

Apparatus that may be employed in the present method, and certain types of products that are prepared thereby, are shown diagrammatically by way of illustration in the accompanying drawing, in which:

Fig. 1 is a vertical section of one form of apparatus for piercing the surface of a sheet in accordance with the method of the present invention;

Fig. 1a is a vertical section of a form of apparatus for treating a rouletted sheet with a penetrant;

Fig. 1b is a fragment of a section of the apparatus shown in Fig. 1 taken on line a—a;

Fig. 2 is a diagrammatic representation of a modification of the apparatus;

Fig. 3 is a fragmentary sectional view of a sheet and rouletting means applied thereto, the rouletting means extending through the sheet from one side to the other;

Fig. 4 is a fragmentary sectional view taken on a plane parallel to and between the sides of a sheet, showing one arrangement of ducts in a sheet, and illustrating the distribution of a penetrant into the body of a sheet from the sides of one of the ducts;

Fig. 5 is a fragmentary sectional view through the thickness of a sheet in which ducts extend part of the way through the sheet;

Fig. 6 is a fragmentary sectional view through the thickness of a laminated sheet in which ducts extend through one of the laminations;

Fig. 7 is a fragmentary plan view of a sheet in which relatively short slits have been made as distinct from openings substantially circular in cross section as shown in Fig. 4;

Fig. 8 is an enlarged fragmentary sectional view through the thickness of a plastic sheet in which ducts and applied penetrant extend part of the way into the body of the sheet; and

Fig. 9 is a diagrammatic representation of a fragment of a floor covering showing ducts and coloring material of figured decorations extending through the thickness of the floor covering and showing the zoning of the different colors making up the figured decorations.

The present method may be applied to various types of sheet materials that are impregnable, or capable of being impregnated. Fibrous sheets prepared from such materials as animal, vegetable or mineral fibers with or without binders are used. Felt, asbestos, wood, or paper sheets, or sheets prepared from certain types of plastic

compositions are satisfactorily employed. The plastic composition may be of the type of a linoleum composition, a plastic wood composition or other plastic with sufficient plastic binder mixed with a fiber or finely ground fiber to be calendered to form a solid though porous sheet.

Plastic sheets are generally considered unsuitable for penetration purposes. Any plastic sheet, whether or not it contains fibers, is suitable for use in the present process, if it is porous, and penetrable with a fluid penetrant used for saturation or decorative purposes. By perforating such a sheet, penetration is obtainable not only from an outer surface but also laterally from the walls of each duct. Since penetration is thus obtained, a smoother surface can be initially provided on a sheet and dependence need not be entirely placed on penetration from such surface only.

The ducts in a sheet may be pin ducts, such as those produced by roulette or other types of hole forming or punch machines. Ducts are also produced by drilling, in which case some of the material of the sheet treated is removed and the ducts later filled with saturant or plastic material to render the ducts invisible. Ducts can be formed by the use of a very fine drill, so fine that the product when in use, as a finished floor covering, for example, will not disclose to the user the individual openings. It is preferable not to remove the material of a sheet when forming the ducts.

Two types of duct forming means are shown by way of example in the accompanying drawing. In Fig. 1, a flat press type is shown wherein the duct forming points 1 extend from the surface of a flat block 2. The duct forming points are either pins or needles preferably of relatively small diameter. They are spaced a predetermined distance apart so that when a penetrant such as a saturant or coloring material is applied to a sheet that has been pierced, the penetrant will spread from the walls of ducts toward adjacent ducts a sufficient distance so the penetrant will meet or overlap between the ducts. In other words, a penetrant applied to the surface of a pierced sheet will pass into the body of the sheet through the ducts and laterally beneath the surface of the sheet for distances greater than or substantially equal to one half the distances between adjacent ducts. As indicated above, the spacing of the ducts depends on the density of the sheet. It also depends on the penetrating qualities of the penetrant. In some cases, it is desirable to pierce only a limited portion of a sheet or to limit the ducts to certain decorative figures in a sheet; but to obtain uniform penetration, the ducts are uniformly spread throughout the entire sheet.

The points 1 extend downwardly from the surface of the block 2 for a distance equal to the thickness of a sheet to be pierced in the event that the ducts are to pass entirely through the sheet as shown in Fig. 3, wherein the surface of the block 2 provided with the points 1 is shown pressed against the surface of a sheet 3. On the other hand, if the points extending from the bottom of block 2 project therefrom a distance less than the thickness of a sheet, ducts such as those shown in Fig. 5 are obtained, which extend only part of the way through a sheet, as shown at 4 in the sheet 5.

If the sheet to be treated is laminated, as shown in Fig. 6, which illustrates a sheet having two

layers 6 and 7, ducts 8 may extend through the upper layer 6 only or through both the layers.

In Fig. 8, which illustrates a porous plastic sheet having a backing 9 and a layer of plastic 10, ducts are shown extending part of the way through the plastic layer. The ducts in such a sheet may, if desired, extend through the plastic layer 10 and also through the backing layer 9. The horizontal lines 11 between the ducts 11 illustrate the substantial depth of penetration of a penetrant (colored blue, for instance) with said ducts extending part of the way through the sheet. In linoleum with a burlap backing, for instance, the coloring material may extend through the burlap so as to show an inlaid effect on the back. As explained in detail hereinbelow, a plastic or other sheet, when provided with figured decorations, may have the same figure or decoration visible on the back of the sheet as on the top. An inlaid effect may be produced with liquid, or plastic, or any filling material.

One means of regulating the distance of penetration of the piercing pins is to apply a sheet or several sheets to the under side of the block 2 and press such sheet or sheets firmly into the spaces between the pins, leaving the points of the pins exposed for a distance equal to the depth of the ducts desired in the sheet.

Referring to Fig. 1, sheet material 12 is extended from a roll (not shown) across the top of a base 13 beneath the piercing means 2. In providing ducts in a sheet such as pasteboard or other paper board, Kraft, or a rag sheet, or other sheet, the sheet is passed underneath the piercing block 2, a distance equal to the width of the block. The block is lowered and the sheet pierced, whereafter the block is raised and separated from the sheet by separating means 14 and 15. The sheet is then passed a further distance equal to the width of the block 2, so that the portion adjacent the previously pierced portion may be pierced.

Instead of block 2, a single row of needles adapted to extend across the sheet may be operated vertically and alternately up and down. The shifting of the sheet and the piercing thereof with the needles may be timed to provide rows of ducts properly spaced apart.

To apply a penetrant to a pierced sheet, the latter may be passed through a block printing machine, rotary printing machine, a saturating machine, a coating machine, or any machine well known in the art for saturating or decorating sheet material.

By way of illustration, the drawing shows (Fig. 1a) a pierced sheet 12 in position for passing through a block printing machine. The sheet is moved on a base 13 underneath blocks 17 and 18 which apply the penetrant. Enough penetrant may be laid on the sheet to fill the ducts and yet have a thin film on the surface of the sheet. For ordinary saturation purposes, the sheet passing over a roll 19 may be passed to a calendering means for the purpose of smoothing the sheet and closing the ducts. When applying figured decorations to a sheet, calendering immediately after passing through a printing machine may be omitted to prevent disfiguring. A sheet is preferably moistened before printing with a material that is compatible with the vehicle of the print paint to promote rapid penetration.

Fig. 4 illustrates the distribution and spacing of ducts 26 in a sheet 24. Fig. 4 also illustrates the spread of a penetrant laterally beneath the surfaces of a sheet from one duct towards the

adjacent ducts as at 22. Ordinarily, as in the case of a hard Krafelt sheet, the ducts 20 may be spaced from one-sixteenth to one-eighth of an inch apart. The spacing of ducts as well as the viscosity of the penetrant varies with the density or absorbency of the sheet.

A penetrant suitable for floor covering purposes may be prepared by grinding from about two to three parts by weight of pigment to one part by weight of oil or vehicle to form a paste. The proportion of oil to pigment depends upon the oil absorption of the pigment. Some pigments require more oil to wet them or to make a paste than other pigments. The above paste is thinned to a suitable consistency with either oil or naphtha in the case of oil paints, and in the case of water paints, thinning may be accomplished with water.

A suitable formula for a green penetrant is as follows:

|              | Pounds |
|--------------|--------|
| Chrome green | 250    |
| Cliffstone   | 200    |

The above mixture is ground with about 210 pounds boiled linseed oil, and the resulting paste thinned down to a proper viscosity.

To produce a blue penetrant, the following formula may be used:

|                  | Pounds |
|------------------|--------|
| Ultramarine blue | 250    |
| Cliffstone       | 200    |

The latter materials are ground with about 220 pounds of boiled oil and the resulting paste thinned to the desired consistency.

For a white penetrant the following formula may be used:

|            | Pounds |
|------------|--------|
| Lithopone  | 375    |
| Cliffstone | 200    |

The latter pigments are ground in about 200 pounds of boiled oil to form a paste which is thinned to a desired consistency.

The viscosity of a penetrant, such as the above paints, may vary from 25 to 35 seconds on a #10 Ford viscosity cup. Such viscosities vary depending on the amount of penetration desired, and on the manner of applying the penetrant. The pigments and oils are also varied, both in composition and in their proportions. The proportions may be varied for reasons other than those indicated above, namely, for the purpose of varying the color obtained in a sheet.

Certain sheets tend to repel penetrants such as coloring materials primarily because of their moisture content. A satisfactory moisture content is below two or three per cent. Some papers have a higher proportion of moisture and are still usable. A "bone dry" paper is desirable, but paper carrying up to or about five per cent of moisture is considered practical for penetration purposes with decorating or other media.

In the use of print blocks 17 and 18, such as those on flat bed machines in floor covering plants, it is not necessary that there shall be any definite relation between the spacing of the lines on a print block and the spacing of the ducts in a sheet. The paint or penetrant is deposited by the wooden lines of a block and the paint thus applied covers the entire surface of the sheet.

In a roller type machine (Fig. 2), a sheet 24 is guided by means 23 between rollers 25 and 26, the roller 25 having metal points 27 distributed over its surface and extending diametrically therefrom, so that when a sheet is passed be-

tween the rollers, it is pierced by the points. The points 27 are long enough to pierce a sheet through its thickness or part of the way through its thickness. The sheet 24, after piercing, is passed between rollers 28 and 29 which may be engraved rollers, or other rollers by which a penetrant may be applied either to the top of the sheet or to the bottom or both. After applying the penetrant, the sheet is passed between calendering rollers 30 and 31 for the purpose of smoothing the sheet and in certain instances for closing the ducts. If figured decorations are applied in or on the sheet, it is desirable to dry the decorating material beyond the tacky stage before calendering.

Various types of saturants or decorative coloring materials may be employed in addition to those referred to above. For instance, dyes and inks may be employed as decorative colorings.

Various saturants including bituminous saturants, may be applied such as asphalts, tar and other bitumens. In the preparation of roofing sheets in which it is essential that the fibrous material employed for this purpose be filled, saturation may be accomplished quickly and thoroughly. A sheet after being pierced may be passed through a saturation tank with or without means for subjecting the saturant to pressure. Under certain conditions plastics or thermoplastics in fluid or melted form are forced into a pierced sheet. Plastic wood or a plastic made from pigment and oil may be used for this purpose. The plastic after entrance into the ducts and pores of a sheet eventually solidifies.

For some purposes it is found desirable to maintain the upper surface of a floor covering, for instance, smooth and fairly dense. In such case the back of the sheet may be pierced and ducts provided in the sheet which pass about three-quarters or four-fifths of the way through the thickness of the sheet without breaking the top surface. The penetrant is then applied to the pierced side of the sheet. By this method, a penetrant of higher viscosity can be used whereby a saving of solvents or other vehicle is realized and a denser sheet is obtainable.

In the preparation of a sheet material in accordance with the present invention, a sheet may be pierced before there are any operations on the sheet or at any stage between operations. If a sheet becomes sealed on its surface by a printing operation, the sheet may then be pierced before a subsequent saturation thereof. If the ducts are large, a plastic material is calendered or pressed into the sheet, forming an inlaid material. In other words, the sheet forms a matrix into which a plastic material can be forced. A sheet to be decorated may be primed or moistened before the decorating material is applied. A sheet may be saturated or surface-treated after the decorating material is applied. It may or may not be calendered or pressed to a smooth surface at any stage during processing. The calendering time depends on the nature of the materials used and the drying time of such materials and also whether or not they are thermoplastic.

Ducts may be any shape in cross section, as, for instance, circular, or substantially so, as shown in Fig. 4, or they may be in the form of slots or slits, as shown in the sheet 32 at '73 (Fig. 7). Depending on the nature of a sheet and the cross section of a piercing means, the ducts when made may be invisible to the naked eye when the goods is used as a floor covering.

In Fig. 9 a sheet having figured decorations, hereinbefore referred to, is illustrated. Decorative figures may extend part of the way through the thickness of a sheet as illustrated in Fig. 8, or all of the way through the thickness of a sheet 35 as shown at 36 and 37. The sheet 35 may be a porous plastic composition provided with a backing such as woven goods 38, or felt or other goods. A linoleum or other floor covering material may be pierced clear through from the top to the bottom of the sheet as shown at 39 to provide for penetration of the various colors, employed in figured decorations, through the thickness of the sheet. Thus, an inlaid effect is produced on the top surface of sheet goods as well as on the bottom surface of the sheet goods. By means of the ducts, the inlaid effect on the bottom surface of the sheet goods is rendered more pronounced.

The present invention has numerous advantages in addition to those referred to above. Less expensive sheet material may be used to start with and by piercing of such sheet material, the latter is rendered more flexible. By piercing, one may use a denser, smoother sheet which does not require so much filling material or top dressing in order to provide a compact, smooth sheet when finished. When applying saturants, penetration is more complete. The ducts serve the purpose of permitting a sheet to be filled with harder and better wear-resisting materials than the composition of the sheet itself. The sheet acts as a skeleton which is filled with the wear-resisting materials. In the preparation of decorative sheets, the ducts make it possible to use a denser and harder sheet and yet make it possible to penetrate the sheet with colorings well down into the sheet or all the way through it.

One of the difficulties in the manufacture of decorative sheets is the preparation of a solid sheet from porous sheet materials. If there are any pores in a floor covering, for instance, after the surface is worn down from use, the worn sheet is more apt to collect dirt. A sheet prepared by the present process is readily rendered solid throughout and free from pores. The more solid a sheet, the more satisfactory it is as a wear surface.

What is claimed is:

1. A method of manufacturing decorative impregnated sheet material, which method comprises piercing a fibrous sheet the surface of which is resistant to impregnation by fluid coloring or toughening penetrants, said piercing providing a multiplicity of minute ducts positioned closely together and extending uniformly across its surface without removing any of the material of the sheet, and applying a fluid decorative medium penetrately to the surface of the sheet in certain prescribed zones to saturate the material of the sheet and extend laterally from each duct, the ducts being so small as to be substantially imperceptible to the eye when the goods is used as a floor covering.

2. A method of manufacturing decorative impregnated sheet material, which method comprises subjecting a sheet the surface of which is resistant to impregnation by fluid coloring or toughening penetrants to pin piercing to provide a multiplicity of minute ducts positioned closely together and extending well down into the body of said sheet, and applying a decorative saturant in figured color decorations to the sheet in certain prescribed zones so as to fill the pin holes and pores in the material of the sheet and extend

laterally from each duct, the ducts being so small as to be substantially imperceptible to the eye when the goods is used as a floor covering.

3. A method of manufacturing decorative impregnated sheet material, which method comprises rouletting a sheet, the surface of which is resistant to impregnation by fluid coloring or toughening penetrants, said rouletting providing a multiplicity of minute ducts positioned closely together and extending well down into the body of said sheet while leaving the surface sufficiently continuous to print upon, and applying a decorative saturant in figured decorations to the sheet to penetrate the sheet therewith and uniformly distribute the saturant in the body of the sheet and laterally from each duct, the ducts being so small as to be substantially imperceptible to the eye when the goods is used as a floor covering.

4. A method of manufacturing decorative impregnated sheet material, which method comprises piercing a fibrous sheet, the surface of which is resistant to impregnation by fluid coloring or toughening penetrants, said piercing providing a multiplicity of minute ducts positioned closely together and extending well into the body of the sheet to provide ducts for introduction of a fluid penetrant into the body of the sheet, the ducts being so spaced that when said fluid penetrant is applied the penetrant entering the ducts and spreading laterally therefrom is uniformly distributed in the body of the sheet while the surface of the sheet remains sufficiently continuous to print upon, and applying a decorative fluid penetrant to the sheet in certain prescribed zones to form figured decorations and causing the penetrant to enter deep down into the ducts and laterally therefrom to the body of the sheet, the ducts being so small as to be substantially imperceptible to the eye when the goods is used as a floor covering.

5. A method of manufacturing a decorative floor covering, which method comprises piercing a porous plastic sheet to provide a multiplicity of minute ducts positioned closely together and extending straight into said sheet for the introduction of a coloring material into the body of the sheet, and applying a coloring medium to the surface of said sheet in the form of figured decorations, and causing said coloring medium to extend into the body of the sheet by penetrating straight into the sheet through said ducts and laterally from said ducts into the pores of the sheet between the ducts to display a figured pattern at the surface of the sheet and to provide substantially the same pattern well down into the body of the sheet, the ducts being so small as to be substantially imperceptible to the eye when the goods is used as a floor covering.

6. A method of manufacturing a decorative floor covering, which method comprises piercing a porous sheet to provide a multiplicity of minute ducts positioned closely together and extending straight into said sheet for introduction of coloring matter into the body of the sheet, and applying coloring matter to said sheet over areas in the form of figured decorations simulating an inlaid structure, causing the said coloring matter to penetrate straight into the sheet through the ducts and laterally from the ducts into the pores of the sheet between the ducts to display a figured pattern at the surface of the sheet and to provide substantially the same pattern well down into the body of the sheet, the ducts being so small as to be substantially imperceptible to the eye when the goods is used as a floor covering.

7. As an article of manufacture, a decorative floor covering comprising a fibrous sheet having a multiplicity of minute ducts positioned closely together and of relatively small cross section, and extending from a surface of the sheet straight into the body thereof for the passage of coloring matter into the body of the sheet, said sheet having been porous prior to impregnation and sufficiently smooth to print upon, said sheet having coloring matter in said ducts and in the pores of the sheet displaying figured decorations extending from one surface of the sheet with substantially the same pattern of figured decoration well down into the body of the sheet, the ducts being so small as to be substantially imperceptible to the user when the goods is used as a floor covering.

8. As an article of manufacture, a decorative covering comprising a pliable sheet having a multiplicity of minute ducts positioned closely together and of relatively small cross section extending from one surface of the sheet straight into the body thereof and said sheet having been porous prior to impregnation and sufficiently smooth to print upon, and coloring matter im-

regnated into the ducts and in the pores of the sheet between the ducts providing an inlaid effect in a pattern appearing on the surface of the sheet and the same pattern extending well down into the body of the sheet, the ducts being so small as to be substantially imperceptible to the eye when the goods is used as a floor covering.

9. As an article of manufacture, a decorative floor covering comprising a fibrous sheet having a multiplicity of minute ducts positioned closely together and of relatively small cross section extending substantially straight through the thickness of the sheet and said sheet having been porous prior to impregnation and sufficiently smooth to print upon, coloring matter in the ducts and in the pores in the sheet throughout the thickness thereof providing an inlaid effect in the pattern visible on the top and extending substantially through to the bottom of the sheet, the ducts being so small as to be substantially imperceptible to the eye when the goods is used as a floor covering.

RALPH G. JACKSON.